

Oct. 5, 1948.

J. W. BAYMILLER

2,450,410

ROLL COVER FOR TEXTILE FIBER DRAFTING

Filed Feb. 27, 1946

*Fig. 1.*



*Fig. 2.*



INVENTOR

John W. Baymiller  
by his attorney  
Stebbins, Clements & Webb.

## UNITED STATES PATENT OFFICE

2,450,410

ROLL COVER FOR TEXTILE FIBER  
DRAFTING

John W. Baymiller, Manheim Township, Lancaster County, Pa., assignor to Armstrong Cork Company, Lancaster, Pa., a corporation of Pennsylvania

Application February 27, 1946, Serial No. 650,609

19 Claims. (Cl. 19—143)

1 Reference is had to the accompanying drawings, in which:

Figs. 1 and 2 are perspective views of roll covers in the form of cots embodying my invention.

This application is a continuation-in-part of my copending applications Serial Nos. 542,880 and 542,881, both filed June 30, 1944, both now abandoned. The invention relates to roll covers or cots for textile fiber drafting machinery used in the drafting of cotton, rayon, worsted and the like fibers. I have discovered that roll covers and cots made of synthetic rubber may be rendered lap-resistant by the incorporation in the synthetic rubber of certain reaction products resulting from the digestion in water dispersion of a protein and a water-ionizable modifying agent which combines with the protein to produce a water-soluble digestion product which is readily dispersible in the synthetic rubber.

The present invention is an improvement on the roll covers and cots described and claimed in my copending application Serial No. 634,230, which was a continuation-in-part of my copending applications Serial Nos. 498,680, filed August 14, 1943; 526,380, filed March 14, 1944; and 542,879, filed June 30, 1944, the last three applications being now abandoned.

In the drafting of cotton, rayon, worsted and like fibers, it has been found that an unusual tendency exists for the fibers to "lap up" around the drafting roll, and the problem is particularly difficult in drafting rayon fibers. This problem exists in varying degrees with all types of roll covers with which I am familiar and tends to reduce substantially the field of usefulness of roll covers.

Many attempts have been made to utilize various materials in the formation of roll covers for textile drafting machinery, such as spinning and drawing frames. Leather is a material frequently used. Its chief disadvantages reside in its cost, susceptibility to wear, prevalence of damage caused by the clearing of lap-ups from its circumference and the frequency with which replacements are necessary. Cork composition roll covers or cots have been used to a considerable degree in the textile industry in place of leather. Their advantages over leather reside in their initial low cost and the length of service each cot is capable of rendering. These two types of cots comprise the vast majority of cots used in the textile industry.

Attempts have been made to utilize oil-resistant synthetic rubbers to form the working surfaces of textile fiber drafting roll covers. Such roll covers

5 have been made of "neoprene" (a polymerized chloroprene) and "Perbunan" (a butadiene acrylonitrile copolymer), two well known oil-resistant synthetic rubbers. These materials, while oil-resistant, do not possess the requisite resistance to lapping up. "Neoprene" is not used in the industry at the present time because of its extreme tendency to lap up. Cots of "Perbunan" have been used to some extent for use with cotton and in certain worsted operations, since only a moderate amount of lapping up is encountered. Such cots are not satisfactory for rayon fibers and certain cotton fibers, for they lap up excessively when used for drafting such fibers. In my copending application Serial No. 634,230, referred to above, I disclosed that synthetic rubber roll covers which would be normally non-resistant to lapping up may be made resistant to lapping up under normal conditions of use by the incorporation therein of an animal protein such as glue, together with certain inorganic electrolytes or water-ionizable inorganic substances such as calcium nitrate, aluminum sulphate, potassium aluminum sulphate, sodium aluminum sulphate, ferric sulphate, potassium ferric sulphate, sodium ferric sulphate, sodium carbonate and phosphoric acid.

10 I have discovered that instead of adding the proteins and the electrolytes as such to synthetic rubber as disclosed in my said prior application Serial No. 634,230, improved results may be secured by digesting a protein with certain water-ionizable modifying agents and incorporating the reaction product resulting from such digestion in the synthetic rubber. I have found that greater lap resistance is attained by the addition of the animal proteins and certain of the inorganic electrolytes described in my copending application if they are digested together previously to their addition to the synthetic rubber. I have also found that effective lapping up resistance is attained at a lower relative atmospheric humidity by the incorporation of the digestion product over that attained by adding the proteins and organic electrolytes as such. I have also discovered that 15 vegetable proteins as well as animal proteins may be used in forming my digestion product, and that certain salts which are not effective when added as such with animal proteins or alone are effective when reacted with protein to form my digestion product.

20 The reaction product which I incorporate into my synthetic rubber roll covers is the product resulting from the digestion in a water dispersion, preferably heated, of a protein and a water-

ionizable modifying agent which combines with the protein to produce a water-soluble digestion product which is readily dispersible in the synthetic rubber. This digestion product is readily ionizable in water and is believed to reduce the electrokinetic potential at the cut surface to substantially zero, as hereinafter more specifically explained under the theory.

The preferred protein is the animal protein glue. Other animal proteins such as casein and gelatin may be used. Vegetable proteins may be used such for example as those derived from soybeans and wheat. I believe that proteins as a class are suitable because proteins as a class may be reacted with the hereinafter described modifying agents to produce a digestion product which is dispersible in the synthetic rubber. The water-ionizable modifying agents which combine with the protein to produce a water-soluble digestion product which is readily dispersible in the synthetic rubber comprise a large number of substances. They have the common property of being water-soluble and ionizable in water and capable of reacting with the protein to produce a water-soluble water-ionizable digestion product which is readily dispersible in the synthetic rubber. The preferred salt for digestion with animal glue is calcium nitrate. Other salts may be used, however, including calcium chloride, sodium nitrate, sodium chloride, sodium sulphate, sodium phosphate and sodium carbonate, as well as the corresponding potassium salts, zinc nitrate, zinc chloride, zinc sulphate, ferric and ferrous chlorides and stannic and stannous chlorides. The substances listed above are common industrial chemicals and are readily obtainable. However, other water-soluble salts may be used which will combine with the protein to produce a water-soluble digestion product which is readily dispersible in the synthetic rubber. Certain salts will not combine with the protein to produce a water-soluble digestion product which is readily dispersible in the synthetic rubber, such for example as the alums, aluminum sulphate, potassium aluminium sulphate and sodium aluminium sulphate, because upon digestion they react with the glue to produce a hardened product which is not water soluble and not readily dispersible in the synthetic rubber. However undigested mixtures of these alums and glue may be used as disclosed in my prior application Serial No. 634,230.

Non-oxidizing acids may be used to form the digestion product with the protein, preferably phosphoric acid. Other non-oxidizing acids are hydrochloric, acetic, citric, tartaric, lactic and maleic. These acids react with the protein to produce a digestion product which is readily dispersible in the synthetic rubber. Acids should be avoided which have an oxidizing effect upon the glue or the synthetic rubber, such as nitric and sulphuric acids.

Bases may also be used to form the digestion product with protein, preferably ammonium hydroxide, which is particularly effective with vegetable proteins. Other bases may be used such as calcium hydroxide, which however is not particularly desirable because of its low solubility.

In making my reaction product a water dispersion or solution is first produced by dispersing or dissolving the protein in water and dissolving the salt, acid or base, in water and mixing the two. The mixture of the water dispersions or solutions of the protein and of the salt acid or base is heated, preferably to a temperature of

about 200 to 212° F. for approximately 1½ to 2 hours. A reaction occurs which produces a digestion product which is distinctly different from the mixture of the original ingredients. For speed in the commercial production of my digestion product, it is preferred to heat to a temperature at or slightly below the boiling point of water. However, the water solution of the ingredients may be heated or warmed to a lower temperature, or even reacted at room temperature, with a correspondingly longer period of time required for digestion. In the case of ammonia, heating tends to evaporate ammonia and the heating should be adjusted to a point of as rapid reaction as can be attained without undue loss from evaporation.

The preferred digestion product is made from glue and calcium nitrate by adding approximately 50 parts of animal glue ("Rex" glue) to 25 parts by weight of water. Parts are given as parts by weight throughout this specification. The glue and water may be placed in a vessel over a water bath until the glue melts. Twenty parts of dry calcium nitrate are dissolved in 20 parts of water and the solution poured into the dispersion of animal protein and the mixture is stirred. The mixture is then permitted to digest for about 1½ hours at a temperature of about 212° F. with occasional stirring to produce a digestion or reaction product which is to be incorporated in the synthetic rubber mix.

When vegetable protein is used, the preferred modifying agent is ammonium hydroxide. Fifty parts of vegetable protein, such as soybean or wheat protein, are mixed with 50 parts of water and stirred to form a water dispersion. About 5 parts of a 28% aqueous solution of ammonia is poured into the protein dispersion and the mixture is stirred. The mixture is then allowed to digest at room temperature for about twenty-four hours with occasional stirring, to produce a digestion or reaction product which is to be incorporated in the synthetic rubber mix.

For convenience in description, I refer to the salts, acids and bases which react with the protein to form the digestion product as "modifying agents." The proportion of modifying agent to protein may be varied over fairly wide limits. The optimum proportion is about 20 parts of modifying agent to about 50 parts of protein. The preferred range is from about 10 to 30 parts of modifying agent to 50 parts of protein. Below such range the beneficial effect of the modifying agent becomes progressively less, although appreciable benefit is observable down to about 5 or even 2½ parts of modifying agent to 50 parts of protein. While it is preferred not to exceed about 30 parts of modifying agent to 50 parts of protein, the modifying agent may be somewhat increased, up to as high as about 40 parts of modifying agent to 50 parts of protein, although at such upper limit some difficulty may be encountered in mixing the digestion product into the synthetic rubber.

The amount of digestion product to be incorporated in the synthetic rubber may vary over fairly wide limits. The optimum proportion of digestion product to the synthetic rubber is about 70 parts of digestion product to 100 parts of rubber. This proportion is figured on the dry weight of the protein and modifying agent. It is in general undesirable to incorporate less than about 20 parts of the digestion product to 100 parts of the synthetic rubber since not enough improvement in lap resistance is en-

countered with a lesser amount. It is preferred to use at least about 40 parts of digestion product to 100 parts of synthetic rubber. The digestion product may be incorporated nearly to the point where it ceases to be the internal phase. However, it is in general inadvisable to incorporate more than about 100 parts of digestion product to 100 parts of synthetic rubber. It is preferred that the digestion product be not more than about 80 parts to 100 parts of the synthetic rubber.

While in the neighborhood of 70 parts of digestion product to 100 parts of synthetic rubber has been found to give excellent results with most synthetic rubbers, the particular percentages may be varied somewhat depending upon the particular synthetic rubber employed. Butadiene acrylonitrile copolymers are somewhat more resistant to lapping up than polymerized chloroprene and isoprene acrylonitrile copolymers and therefore the amount of the digestion product required for the butadiene acrylonitrile copolymers may be reduced somewhat beyond that for polymerized chloroprene and isoprene acrylonitrile copolymers.

By the term "synthetic rubber" I mean those synthetic substances which are commonly referred to as "synthetic rubbers" and which have

results were obtained with a humidity differential existing between desiccated air and air of 80% relative humidity at 70° F.:

- 5 "Chemigum N-1"— $2.2 \times 10^{-3}$  grms. per sq. cm. per day  
 "Perbunan"— $1.5 \times 10^{-3}$  grms. per sq. cm. per day  
 "Hycar OR-15"— $1.0 \times 10^{-3}$  grms. per sq. cm. per day  
 10 "Neoprene GN"— $0.8 \times 10^{-3}$  grms. per sq. cm. per day

15 While my tests show that synthetic rubbers of the butadiene acrylonitrile copolymer type, the polymerized chloroprene type, and the isoprene acrylonitrile copolymer type are satisfactory, I believe that any synthetic rubber having the characteristics above indicated may be employed.

20 As contrasted with synthetic rubbers having the characteristics above indicated as essential for satisfactory operation, there are synthetic rubbers of the "butyl" and "Vinylite" types which are not satisfactory because they cannot be vulcanized, or are not sufficiently oil-resistant, or are subject to excessive cold flow because of their thermoplastic nature.

25 Reference is now made to the following examples in which the proportions of the various ingredients are given by weight:

|                                                                                                       | I   | II  | III | IV  | V   | VI  | VII | VIII | IX  | X   | XI  | XII |
|-------------------------------------------------------------------------------------------------------|-----|-----|-----|-----|-----|-----|-----|------|-----|-----|-----|-----|
| "Hycar".....                                                                                          | 100 |     |     | 100 |     |     | 100 |      |     | 100 |     |     |
| "Chemigum".....                                                                                       |     | 100 |     |     | 100 |     |     | 100  |     |     | 100 |     |
| "Perbunan".....                                                                                       |     |     | 100 |     |     |     |     |      |     |     |     | 100 |
| Cork particles 20/30 mesh.....                                                                        |     |     | 50  |     |     |     |     | 50   |     |     | 50  | 50  |
| Digestion Product of 50 Parts Animal Glue and 20 Parts Calcium Nitrate calculated on dry weights..... | 70  | 70  | 70  |     |     |     | 70  | 70   | 70  |     |     |     |
| Digestion Product of 50 Parts Animal Glue and 20 Parts Phosphoric Acid calculated on dry weights..... |     |     |     | 70  | 70  | 70  |     |      |     | 70  | 70  | 70  |
| Sulfur.....                                                                                           | 10  | 10  | 10  | 10  | 10  | 10  | 10  | 10   | 10  | 10  | 10  | 10  |
| Titanium dioxide.....                                                                                 | 15  | 15  | 15  | 15  | 15  | 15  | 15  | 15   | 15  | 15  | 15  | 15  |
| Triacetin.....                                                                                        | 10  | 10  | 10  | 10  | 10  | 10  | 10  | 10   | 10  | 10  | 10  | 10  |
| Benzothiazyl disulfide.....                                                                           | 1.5 | 1.5 | 1.5 | 1.5 | 1.5 | 1.5 | 1.5 | 1.5  | 1.5 | 1.5 | 1.5 | 1.5 |
| Carbon black.....                                                                                     | 0.3 | 0.3 | 0.3 | 0.3 | 0.3 | 0.3 | 0.3 | 0.3  | 0.3 | 0.3 | 0.3 | 0.3 |
| Zinc oxide.....                                                                                       | 5   | 5   | 5   | 5   | 5   | 5   | 5   | 5    | 5   | 5   | 5   | 5   |

physical properties resembling those of natural rubber, as set forth, for example, in the definition of synthetic rubber appearing on pages 3 to 4 of the circular C427 of the United States Department of Commerce entitled "Synthetic rubber: A Review of Their Compositions, Properties, and Uses," by Lawrence A. Wood, issued June 25, 1940; and on page 9 of "Natural and Synthetic Rubbers," by Harry L. Fisher, being the Edgar Marburg lectures of 1941 presented before the forty-fourth annual meeting of the American Society for Testing Materials.

My tests have been carried out primarily with synthetic rubbers of the following types: butadiene acrylonitrile copolymers, of which "Perbunan," "Chemigum" and "Hycar" are commercial examples, and which contain varying percentages of acrylonitrile; chloroprene polymer, of which "neoprene" is a commercial example; and isoprene acrylonitrile copolymers, which have been made experimentally. These have all proved satisfactory synthetic rubber bases for lap-resistant cots when mixed with my digestion product. These synthetic rubbers have certain common characteristics which adapt them for use in covers for textile drafting rolls. They are vulcanizable. When vulcanized they are oil-resistant, resilient and non-thermoplastic. When vulcanized they are all water permeable to a certain extent, as indicated by the following tests, the results of which are expressed in the terms used by the American Society for Testing Materials in Methods for Water Vapor Permeability, in which the

45 In place of the digestion products formed from glue and a salt and glue and an acid, the digestion product in the same amount formed by digesting a protein, either a vegetable or an animal protein with ammonium hydroxide, may be used.

50 In the above compounds, "Hycar," "Chemigum," and "Perbunan" are synthetic rubbers of the acrylonitrile butadiene copolymer type containing about 40%, 30% and 26% respectively of acrylonitrile. The cork particles are included in the composition to aid in resistance to eyebrowning. In the specific examples the glue was

55 Cudahy Packing Company's "Rex" glue, although other commercial glues may be employed, such as Swift's "Economy" glue, "Peter Cooper AA" glue, etc.

60 Sulfur, of course, is the vulcanizing agent; titanium dioxide and carbon black are used primarily as pigments. If desired, other pigments and fillers may be included in the above compositions. Triacetin is used as a softener or plasticizer and other plasticizers may be used in its place, for example, tricresyl phosphate or dibutyl phthalate or dibenzyl ether. Benzothiazyl disulfide (Altax) is a conventional accelerator and, of course, other accelerators may be used with satisfactory results. Zinc oxide is used primarily

65 as an activator for the accelerator.

70 The synthetic rubber is milled on any suitable rubber mill until it is satisfactory for use, then my digestion product is milled into the rubber at a suitable temperature. In milling my digestion product into the synthetic rubber, it is de-

sirable that the digestion product be milled into the rubber on a warm mill. The mill should be warm but must not be too hot for if it to be too hot, the water may evaporate from the digestion product prematurely so that the digestion product may adhere to the rolls of the rubber mill. After the digestion product has been thoroughly dispersed in the synthetic rubber mix the milling is continued, preferably with heat applied to the mill rolls until the water contained in the digestion product has been largely driven off. The digestion product is readily dispersible in the synthetic rubber and is used in an amount to form the dispersed or internal phase. When the digestion product has been thoroughly milled into the synthetic rubber it is uniformly dispersed therein so that the mixture has the appearance of a homogeneous solution. When a thin sheet of the milled rubber is viewed in front of a light it has nearly the same transparent appearance as the untreated synthetic rubber. There are no discrete particles of the digestion product observable to the naked eye or even under 150 magnifications. The remaining ingredients should be added to the mass after the digestion product has been uniformly dispersed throughout the rubber. They may be added to the milled mass as is customary and well-known in the industry.

The synthetic rubber compound so prepared is then sheeted or tubed by means of any suitable tubing device. If the compound be sheeted, it is rolled about a mandrel to form a cot. If the compound be tubed, the tube is slipped on the mandrel. In either case, the cot stock disposed about the mandrel is wrapped with wet fabric tape and cured with open steam. The temperature and duration of the cure may be varied in accordance with standard vulcanizing practice. For the above compounds, a curing time of 55 minutes at 300° F. is generally satisfactory.

After the curing operation the tubes are removed from the mandrel, the fabric tape is removed, and the tubes are buffed or ground to obtain a satisfactory surface, are cut to size to form cots, and bevelled, if desired. Cots so formed may be supplied to spinning mills or, if desired, may be mounted on spinning rolls at the place of manufacture.

It appears that the capacity of my digestion product to absorb water is considerably increased over that of the protein alone. One advantage of my digestion product resides in the fact that many materials which are not sufficiently compatible with rubber to be milled therein and dispersed satisfactorily through the synthetic rubber may be digested with the protein and the digestion product so formed is easily and readily milled into the rubber. For example, calcium chloride is not satisfactory for decreasing the lap resistance of a synthetic roll cover when incorporated alone or as an undigested mixture with animal glue, but is found to be a highly satisfactory salt for use when digested with protein as above described. Other materials which are unsatisfactory if used alone or in an unreacted mixture with animal protein are sodium chloride, sodium nitrate, trisodium phosphate, citric acid, lactic acid, tartaric acid and maleic acid. These materials, however, are very satisfactory modifying agents for digestion with proteins.

My digestion products are compatible with the synthetic rubber in which they are incorporated and do not deleteriously affect the synthetic rubber mix.

Suitable compounds embodying polymerized chloroprene are as follows:

|    |                                                                                                  | XIII | XIV | XV  | XVI |
|----|--------------------------------------------------------------------------------------------------|------|-----|-----|-----|
| 5  | "Neoprene GN"                                                                                    | 100  | 100 | 100 | 100 |
|    | Cork particles 2/30 mesh                                                                         | 42   |     |     | 42  |
|    | Digestion Product of 50 Parts Animal Glue and 20 Parts Calcium Nitrate calculated on dry weights | 70   |     |     | 70  |
| 10 | Digestion Product of 50 Parts Animal Glue and 20 Parts Phosphoric Acid calculated on dry weights | 70   | 70  | 70  |     |
|    | Light magnesia                                                                                   | 4    | 4   | 4   | 4   |
|    | Stearic acid                                                                                     | 3    | 3   | 3   | 3   |
|    | Titanium dioxide                                                                                 | 15   | 15  | 15  | 15  |
|    | Graphite                                                                                         | 2.6  | 2.6 | 2.6 | 2.6 |
| 15 | Neozone A                                                                                        | 2    | 2   | 2   | 2   |
|    | Zinc oxide                                                                                       | 5    | 5   | 5   | 5   |

In place of the digestion products formed from glue and a salt and glue and an acid, the digestion product in the same amount formed by digesting a protein, either a vegetable or an animal protein with ammonium hydroxide, may be used.

These materials may be compounded in the same manner as described with regard to acrylonitrile butadiene copolymers and the cot may be formed in the same manner. The light magnesia is used as a curing agent. In its place I may use litharge or lead dioxide. Stearic acid is used as a lubricant and, if desired, paraffin may be used in its place. Neozone A is an anti-oxidant and any suitable anti-oxidant may be used. Zinc oxide is used primarily as a curing agent.

The following compounds illustrate my invention as applied to the manufacture of cots made from isoprene acrylonitrile copolymers:

|    |                                                                                                 | XVII | XVIII | XIX | XX  |
|----|-------------------------------------------------------------------------------------------------|------|-------|-----|-----|
|    | Isoprene acrylonitrile copolymer                                                                | 100  | 100   | 100 | 100 |
|    | Cork particles 20/30 mesh                                                                       | 50   |       |     | 50  |
| 40 | Digestion Product of 50 Parts Animal Glue and 20 Parts Calcium Nitrate calculated on dry weight | 70   | 70    |     |     |
|    | Digestion Product of 50 Parts Animal Glue and 20 Parts Phosphoric Acid calculated on dry weight | 70   | 70    | 70  | 70  |
|    | Titanium dioxide                                                                                | 15   | 15    | 15  | 15  |
|    | Triacetin                                                                                       | 10   | 10    | 10  | 10  |
|    | Carbon Black                                                                                    | 0.3  | 0.3   | 0.3 | 0.3 |
| 45 | Sulfur                                                                                          | 10   | 10    | 10  | 10  |
|    | Benzothiazyl disulfide                                                                          | 2    | 2     | 2   | 2   |

In place of the digestion products formed from glue and a salt and glue and an acid, the digestion product in the same amount formed by digesting a protein, either a vegetable or an animal protein with ammonium hydroxide may be used.

Cork granules may be included in any of these various synthetic rubber mixes. The presence of the cork granules improves the "eyebrow" resistance, particularly of cots of the chloroprene type.

An "eyebrow" may be defined as a collection of waste fibers pulled from the roving by the cot which is not carried rearwardly of the clearer board by the rotating cot and which accumulate at the front of the clearer board in a bunch-like formation. As the eyebrow increases in size, it is occasionally pulled from the clearer board by the roving been spun and causes a hard spot in the yarn which is called a "nub."

The cork granules may be included in various quantities. I have found that the amount of cork granules included in the various mixes may fall within the range of 25 to 125 parts to each 100 parts of the synthetic rubber mix. The cork granules may vary as to particle size. For most satisfactory results the cork granules should not be larger than about 10 mesh or smaller than about 50 mesh and I have found that particularly good

results are obtained with cork granules falling within the range of 20 to 30 meshes to the inch United States Standard sieves. The cork granules are preferably added along with the other ingredients which are incorporated in the synthetic rubber on the rubber mill and are thus uniformly distributed in the synthetic rubber mix so that there is a uniform distribution of such particles at the working surface.

Granules or particles of other materials which minimize eyebrowning may be similarly employed in place of cork. Such materials include wood flour, fine mesh sand, preferably about 100 mesh, organic filler particles of a nature similar to cork such as soft wood, balsa, etc., as well as other materials which minimize eyebrowning.

I believe that the failure of the synthetic rubber cots as heretofore produced without being modified by an effective amount of a water-ionizable electrolyte may be explained as follows: A certain amount of water is adsorbed upon the surface of a cot, particularly under the operating conditions of modern textile mills where a relatively high humidity, usually about 60%, is maintained to prevent accumulation of static charges and to render the fibers more amenable to drafting. I believe that such water forms a Helmholtz electric double layer upon the surface of the cot and, in the case of synthetic rubber compounds, the rubber surface has an electrokinetic or zeta potential negative with respect to the moisture film. Such electrokinetic or zeta potential is described in "Electrokinetic Phenomena," Abramson, 1934; "Outlines of Biochemistry," Gortner, second edition, 1938, pages 147-150; "Physical Chemistry," MacDougall, revised edition, 1943, pages 686-694.

The fibers also have a certain amount of water adsorbed on their surfaces so that I believe that there is present on the fibers also a Helmholtz double layer with the surface of the fiber having a zeta potential negative with respect to the adsorbed water film. There is thus a zeta potential set up in the cot-water interface and another zeta potential set up at the fiber-water interface resulting in firm adhesion of water to both the synthetic rubber and fiber. When the two are pressed firmly together, as in the drawing operation, the water film becomes common to both the cot and the fiber and the forces of cohesion in the water itself tend to bond or cement together the cot and fiber, thus causing lapping of the fiber around the cot. I believe that this theory acceptably explains the lapping up action which occurs with the usual synthetic rubber cots of commerce. While I believe that the electrokinetic theory offers the best explanation of the phenomena which I have observed, it is to be understood that the invention is not to be limited to the theory.

I believe that the non-lapping characteristics imparted to synthetic rubber cots by the incorporation of my water-ionizable digestion product is due to the fact that the digestion product in the synthetic rubber-electrolyte mixture supplies the necessary electric charges to reduce the zeta potential at the cot-water interface or the fiber-water interface to zero or substantially zero, thereby destroying the adhesion between the cot and the fibers and thus preventing lapping. The zeta or electrokinetic potential theory is set forth in greater detail in my copending application Serial No. 634,230, to which reference is made.

I have also found that moisture should be present at the surface of the cot, at least to the extent normally present under operating conditions in textile mills. Experiments have been

carried out wherein synthetic rubber cots containing my digestion product have been prepared under extremely dry conditions, that is, they have been dried on the rubber mill at a high temperature, vulcanized in a hot air oven at 300° F., and kept stored in a desiccator after they have been prepared. Even though they contained my digestion product, the cots lapped up badly. When the same synthetic rubber-digestion product composition cots were exposed to the usual humid atmosphere of a textile mill, or dipped in water and the surface wiped free of water, the cot functioned very well with regard to lapping. I believe that the presence of a certain amount of moisture is required to bring the electrolytic digestion product into water solution where its charges are effective in reducing the zeta potential.

I have further found that while some moisture is required to make the synthetic rubber cots described in this application effectively non-lapping, the amount of moisture thus required is substantially less than that required for rendering non-lapping the cots described in my earlier copending application Serial No. 634,230, and that the non-lapping characteristics of the cots disclosed in this application are enhanced over those disclosed in my said prior application at the same relative humidities.

I have also found that the effectiveness of my digestion product in synthetic rubber cots where moisture is present is related to the water vapor permeability of the vulcanized synthetic rubber. For instance, "Chemigum N-1" has the highest water vapor permeability of the synthetic rubbers with which I have experimented. "Perbunan" has the next highest permeability and is followed by "Hycar OR-15," "neoprene GN" and a special isoprene acrylonitrile copolymer, which is made experimentally, in the order named. I have found that the higher the permeability of the synthetic rubber containing my electrolytic digestion product, the better the resistance to lapping. I offer as a possible theoretical explanation of these observations that the electrolytic digestion product incorporated into the synthetic rubber is more readily available at the surface in the case of the synthetic rubber having the greater water vapor permeability.

In the drawings, Fig. 1 is a perspective view of a roll cover embodying my invention; and Fig. 2 is a similar view of such roll cover including cork granules.

While I have disclosed certain preferred embodiments of my invention, it will be understood that my invention is not limited thereto but may be otherwise embodied and practiced within the scope of the following claims.

I claim:

- 60 1. A lap-resistant roll cover for textile fiber drafting having a working surface made of a vulcanized oil-resistant resilient non-thermoplastic somewhat water vapor permeable synthetic rubber which is normally non-resistant to lapping up, having uniformly dispersed therein as the dispersed phase an effective amount of the reaction product resulting from the digestion in water dispersion of a protein and a water-ionizable modifying agent which does not deleteriously affect the protein or the synthetic rubber and combines with the protein to produce a compatible water-soluble digestion product which is readily dispersible in the synthetic rubber, whereby the roll cover is rendered lap-resistant.
- 65 2. A lap-resistant roll cover for textile fiber

11

11  
drafting having a working surface made of a vulcanized oil-resistant resilient non-thermoplastic somewhat water vapor permeable synthetic rubber which is normally non-resistant to lapping up, having uniformly dispersed therein as the dispersed phase from 20 to 100 parts per 100 parts of the synthetic rubber of the reaction product resulting from the digestion in water dispersion of a protein and from 5 to 40 parts per 50 parts of protein of a water-ionizable salt which does not deleteriously affect the protein or the synthetic rubber and combines with the protein to produce a compatible water-soluble digestion product which is readily dispersible in the synthetic rubber whereby the roll cover is rendered lap-resistant.

3. A lap-resistant roll cover for textile fiber drafting having a working surface made of a vulcanized oil-resistant resilient non-thermoplastic somewhat water vapor permeable synthetic rubber which is normally non-resistant to lapping up, having uniformly dispersed therein as the dispersed phase from 20 to 100 parts per 100 parts of the synthetic rubber of the reaction product resulting from the digestion in water dispersion of a protein and from 5 to 40 parts per 50 parts of protein of a water-ionizable non-oxidizing acid which does not deleteriously affect the protein or the synthetic rubber and combines with the protein to produce a compatible water-soluble digestion product which is readily dispersible in the synthetic rubber, whereby the roll cover is rendered lap-resistant.

4. A lap-resistant roll cover for textile fiber drafting having a working surface made of a vulcanized oil-resistant resilient non-thermoplastic somewhat water vapor permeable synthetic rubber which is normally non-resistant to lapping up, having uniformly dispersed therein as the dispersed phase from 20 to 100 parts per 100 parts of the synthetic rubber of the reaction product resulting from the digestion in water dispersion of a protein and from 5 to 40 parts per 50 parts of protein of a water-ionizable base which does not deleteriously affect the protein or the synthetic rubber and combines with the protein to produce a compatible water-soluble digestion product which is readily dispersible in the synthetic rubber, whereby the roll cover is rendered lap-resistant.

5. A lap-resistant roll cover for textile fiber drafting having a working surface made of a vulcanized oil-resistant resilient non-thermoplastic somewhat water vapor permeable synthetic rubber which is normally non-resistant to lapsing up, having uniformly dispersed therein as the dispersed phase an effective amount of the heat reaction product resulting from the digestion in a heated water dispersion of a protein and a water-ionizable modifying agent which does not deleteriously affect the protein or the synthetic rubber and combines with the protein to produce a compatible water-soluble digestion product which is readily dispersible in the synthetic rubber, whereby the roll is rendered lap-resistant.

6. A lap-resistant roll cover for textile fiber drafting having a working surface made of a vulcanized oil-resistant resilient non-thermoplastic somewhat water vapor permeable synthetic rubber which is normally non-resistant to lapping up, having uniformly dispersed therein as the dispersed phase from 20 to 100 parts per 100 parts of the synthetic rubber of the reaction product resulting from the digestion in water dispersion of a protein and from 5 to 40 parts of calcium

12

nitrate per 50 parts of protein, whereby the roll cover is rendered lap-resistant.

7. A lap-resistant roll cover for textile fiber drafting having a working surface made of a vulcanized oil-resistant resilient non-thermoplastic somewhat water vapor permeable synthetic rubber which is normally non-resistant to lapping up, having uniformly dispersed therein as the dispersed phase from 20 to 100 parts per 100 parts of the synthetic rubber of the reaction product resulting from the digestion in water dispersion of a protein and from 5 to 40 parts of phosphoric acid per 50 parts of protein, whereby the roll cover is rendered lap-resistant.

15 8. A lap-resistant roll cover for textile fiber drafting having a working surface made of a vulcanized oil-resistant resilient non-thermo-plastic somewhat water vapor permeable synthetic rubber which is normally non-resistant to  
20 lapping up, having uniformly dispersed therein as the dispersed phase from 20 to 100 parts per 100 parts of the synthetic rubber of the reaction product resulting from the digestion in water dispersion of a protein and from 5 to 40 parts of ammonium hydroxide per 50 parts of protein, whereby the roll cover is rendered lap-resistant.

which the roll cover is rendered lap-resistant.

9. A lap-resistant roll cover for textile fiber drafting having a working surface made of a vulcanized oil-resistant resilient non-thermoplastic somewhat water vapor permeable synthetic rubber which is normally non-resistant to lapping up, having uniformly dispersed therein in an amount between 20 and 100 parts per 100 parts of the synthetic rubber of the reaction product resulting from the digestion in water dispersion of a protein and from 5 to 40 parts per 50 parts of the protein of a water-ionizable modifying agent which does not deleteriously affect the protein or the synthetic rubber and combines with the protein to produce a compatible water-soluble digestion product which is readily dispersible in the synthetic rubber, whereby the roll cover is rendered lap-resistant.

45 10. A lap-resistant roll cover for textile fiber drafting having a working surface made of a vulcanized oil-resistant resilient non-thermoplastic somewhat water vapor permeable synthetic rubber which is normally non-resistant to lapping up, having uniformly dispersed therein as the dispersed phase from about 40 to about 80 parts per 100 parts of the synthetic rubber of the reaction products resulting from the digestion in water dispersion of a protein and from 10 to 30 parts per 50 parts of protein of a water-ionizable modifying agent which does not deleteriously affect the protein or the synthetic rubber and combines with the protein to produce a compatible water-soluble digestion product which is readily dispersible in the synthetic rubber, whereby the roll cover is rendered lap-resistant.

11. A lap-resistant roll cover for textile fiber drafting having a working surface made of a synthetic rubber selected from the class consisting of rubber-like butadiene acrylonitrile copolymers, polymerized chloroprene and isoprene acrylonitrile copolymers, having uniformly dispersed therein as the dispersed phase an effective amount of the reaction product resulting from the digestion in water dispersion of a protein and a water-ionizable modifying agent which does not deleteriously affect the protein or the synthetic rubber and combines with the protein to produce a compatible water-soluble digestion product which is readily dispersible in the syn-

13

thetic rubber, whereby the roll cover is rendered lap-resistant.

12. A lap-resistant roll cover for textile fiber drafting having a working surface made of a rubber-like butadiene acrylonitrile copolymer having uniformly dispersed therein as the dispersed phase an effective amount of the reaction product resulting from the digestion in water dispersion of a protein and a water-ionizable modifying agent which does not deleteriously affect the protein or the synthetic rubber and combines with the protein to produce a compatible water-soluble digestion product which is readily dispersible in the synthetic rubber, whereby the roll cover is rendered lap-resistant.

13. A lap-resistant roll cover for textile fiber drafting having a working surface made of a vulcanized oil-resistant resilient non-thermoplastic somewhat water vapor permeable synthetic rubber which is normally non-resistant to lapping up, having uniformly dispersed therein as the dispersed phase an effective amount of the reaction product resulting from the digestion in water dispersion of glue and a water-ionizable modifying agent which does not deleteriously affect the protein or the synthetic rubber and combines with the glue to produce a compatible water-soluble digestion product which is readily dispersible in the synthetic rubber, whereby the roll cover is rendered lap-resistant.

14. A lap-resistant roll cover for textile fiber drafting in accordance with claim 1, having cork granules uniformly distributed in the synthetic rubber mix at the working surface.

15. A lap-resistant roll cover for textile fiber drafting in accordance with claim 1, having particles of a material which minimizes eyebrowning uniformly distributed in the synthetic rubber mix at the working surface.

16. A lap-resistant roll cover for textile fiber drafting having a working surface made of a rubber-like butadiene acrylonitrile copolymer having uniformly dispersed therein as the dispersed phase from 40 to 80 parts per 100 parts of the synthetic rubber of the reaction product resulting from the digestion in a heated water disper-

sion of glue and from 10 to 30 parts of calcium nitrate per 50 parts of glue, whereby the roll cover is rendered lap-resistant.

17. A lap-resistant roll cover for textile fiber drafting having a working surface made of a vulcanized oil-resistant resilient nonthermoplastic somewhat water vapor permeable synthetic rubber which is normally nonresistant to lapping up, having uniformly dispersed therein as the dispersed phase from 20 to 100 parts per 100 parts of the synthetic rubber of the reaction product resulting from the digestion in a water dispersion of glue and from 5 to 40 parts per 50 parts of glue of a water-ionizable modifying agent which does not deleteriously affect the glue or the synthetic rubber and combines with the glue to produce a compatible water-soluble digestion product which is readily dispersible in the synthetic rubber, whereby the roll cover is rendered lap-resistant.

18. A lap-resistant roll cover for textile fiber drafting in accordance with claim 9, having cork granules uniformly distributed in the synthetic rubber mix at the working surface.

19. A lap-resistant roll cover for textile fiber drafting in accordance with claim 9, having particles of a material which minimizes eyebrowning uniformly distributed in the synthetic rubber mix at the working surface.

JOHN W. BAYMILLER.

## REFERENCES CITED

The following references are of record in the file of this patent:

## UNITED STATES PATENTS

|    | Number    | Name    | Date          |
|----|-----------|---------|---------------|
| 35 | 1,988,491 | Hazell  | Jan. 22, 1935 |
|    | 2,010,012 | Collins | Aug. 6, 1935  |
|    | 2,012,223 | Cutler  | Aug. 20, 1935 |
|    | 2,304,656 | Rockoff | Dec. 8, 1942  |

## FOREIGN PATENTS

|    | Number | Country       | Date |
|----|--------|---------------|------|
| 40 | 3,686  | Great Britain | 1898 |

**Certificate of Correction**

**Patent No. 2,450,410.**

**October 5, 1948.**

**JOHN W. BAYMILLER**

It is hereby certified that errors appear in the printed specification of the above numbered patent requiring correction as follows:

Column 1, line 7, for the word "filled" read *filed*; column 2, line 29, after "such to" insert *the*; column 7, line 3, after "if it" strike out "to"; column 8, line 65, for "been" read *being*; column 9, line 31, for "electrokenitic" read *electrokinetic*; line 51, after "cot and" insert *the*; line 58, for "not be" read *not to*; column 11, line 65, claim 5, after "roll" insert *cover*; column 12, line 53, claim 10, for "products" read *product*; and that the said Letters Patent should be read with these corrections therein that the same may conform to the record of the case in the Patent Office.

Signed and sealed this 15th day of March, A. D. 1949.

**[SEAL]**

**THOMAS F. MURPHY,  
*Assistant Commissioner of Patents.***